

Patented July 14, 1925.

1,545,498

# UNITED STATES PATENT OFFICE.

JAMES D. KLINGER AND CLETE L. BOYLE, OF DETROIT, MICHIGAN, ASSIGNEES TO  
CHEMICAL PRODUCTS CORPORATION, OF DETROIT, MICHIGAN.

## METHOD OF CLEANING STEEL AND IMPARTING RUST-INHIBITIVE PROPERTIES THERETO AND SOLUTION THEREFOR.

No Drawing.

Application filed May 18, 1924. Serial No. 713,778.

To all whom it may concern:

Be it known that we, JAMES D. KLINGER and CLETE L. BOYLE, citizens of the United States, residing at Detroit, county of Wayne, State of Michigan, have invented a certain new and useful Improvement in Methods of Cleaning Steel and Imparting Rust-Inhibitive Properties Thereto and Solution Therefor, and declare the following to be a full, clear, and exact description of the same, such as will enable others skilled in the art to which it pertains to make and use the same.

This invention relates to an improved method of cleaning steel and imparting rust inhibitive properties thereto, and the object of our invention is to provide an improved method and agent by means of which steel may be cleaned and rust inhibitive properties may be imparted to the metal.

More specifically, an object is to provide a cheap, inexpensive, rapid process for removing oil, grease, dirt, rust, etc., from the surface of steel, such as for example, the sheet steel generally employed in the manufacture of automobile bodies, and at the same time imparting to the surface of the steel rust inhibitive properties which will prevent the steel from subsequently corroding and rusting.

Our improved method for treating steel and solution employed therein is particularly useful in preparing the metal for painting. By following this process the steel is thoroughly cleaned so as to receive and retain a priming coat of paint and the surface of the metal is rendered substantially immune to the action of rust either before or following the painting.

We have found that by using a soluble salt of chromic acid, such as potassium chromate or sodium chromate, in our cleaning solution that the rust inhibitive properties of the chromate prevent the steel from subsequent rusting. We provide a cleaning solution containing a small percentage of a rust-attacking and removing acid, such as sulphuric acid, and in order to allow for the successful action of the sulphuric acid and the chromic acid salt on the steel a suitable solvent for the oil and grease and for the removal of dirt is employed. In this case we use an alcohol or acetone. It has been found that denatured alcohol containing a small

amount of acetone performs very satisfactorily.

We have found that an admixture of chromic acid or any soluble salt thereof or any soluble compound containing chromium with sulphuric acid, hydrochloric acid, nitric acid, or such other acid as possesses the property of attacking and removing rust from metal will serve to impart to the surface of the metal when cleaned by the rust-removing acid, rust-resisting qualities, and that this process is particularly valuable as a treatment for metal preparatory to painting the metal.

We prefer to employ a fluid mixture of potassium or sodium chromate, sulphuric acid, denatured alcohol, and acetone. This solution when applied to the metal will remove all oil, dirt, grease, rust, etc., and give the surface of the metal a bright, clean finish and impart thereto rust resisting properties. This solution may be applied to the metal with a brush, sponge, spray, or in any other suitable manner. It may be applied either hot or cold. It has been found that if the rust is deep-seated a hot solution will act more quickly than a cold solution. As a further aid in removing deep-seated rust after the solution has been applied to the metal the badly rusted spots may be rubbed with emery cloth or other similar abrasive.

The following method has been found suitable for use in connection with preparing the sheet steel employed in automobile body construction:

The metal is painted or sprayed with the cleaning solution. In cases where there is deep-seated rust on the steel the cleaning action is accelerated by rubbing the rusty spots with emery cloth or a suitable abrasive, care being taken to keep the spot wet with the cleaning solution. A period of two to three minutes is allowed for the solution to act. The cleaning solution and the resultant products of the cleaning action are then washed from the steel by rinsing with hot or cold water. If cold water is used it should be flowed on freely and the water remaining on the surface blown off with air. If hot water is used any water that has not evaporated should be blown off with air. The method for proceeding from this point is to torch off around mouldings or

pockets with a gas flame, when cleaning automobile bodies, to drive out water. The steel should then be wiped with a cloth saturated with turpentine or alcohol and placed 5 in a pre-heat oven to dry. The steel is then ready for the priming coat of paint.

The strength of the solution may be varied depending upon the work to be accomplished. A solution of the following 10 ingredients in the proportions set forth has been found very satisfactory: four parts of an aqueous solution of potassium or sodium chromate (strength of solution 5%), one-half of one part of concentrated sulphuric 15 acid, four and one-half parts of denatured alcohol, and one part of acetone.

What we claim is:

1. The method of cleaning steel and imparting thereto rust inhibitive properties 20 consisting in treating the metal with a solution containing a soluble salt of chromic acid, sulphuric acid, and an alcohol.

2. The method of cleaning steel and imparting rust inhibitive properties thereto 25 which consists in treating the metal with a solution containing sulphuric acid, a soluble chromate, an alcohol, and acetone.

3. The method of cleaning steel and imparting thereto rust inhibitive properties 30 which consists in treating the metal with a solution containing sulphuric acid, a soluble chromate, and acetone.

4. The method of cleaning steel and imparting thereto rust inhibitive properties 35 which consists in treating the metal with a solution containing potassium chromate, sulphuric acid, and an alcohol.

5. The method of cleaning steel and imparting thereto rust inhibitive properties 40 which consists in treating the metal with

a solution containing sodium chromate, sulphuric acid, and an alcohol.

6. The method of cleaning steel and imparting rust inhibitive properties thereto which consists in treating the metal with a 45 solution composed of denatured alcohol, an aqueous solution of a soluble chromate, and a relatively small percentage of sulphuric acid.

7. A solution to be used in the cleaning 50 of steel and the imparting of rust inhibitive properties to the surface thereof containing the following ingredients in the approximate volume of four parts of an aqueous solution of a soluble chromate, four and a 55 half parts of an alcohol, one part of acetone, and one-half of one part sulphuric acid.

8. A solution to be used for cleaning steel and imparting rust inhibitive properties 60 thereto containing an alcohol, a rust-removing acid, and a solution of a soluble salt of chromic acid.

9. A solution to be used in the cleaning 65 of steel and the imparting of rust inhibitive properties thereto comprising denatured alcohol, acetone, sulphuric acid, and an aqueous solution of a salt of chromic acid.

10. A solution to be used in the cleaning 70 of steel and the imparting of rust inhibitive properties thereto containing an alcohol, sulphuric acid, and potassium chromate.

11. A solution to be used in the cleaning 75 of steel and the imparting of rust inhibitive properties thereto containing an alcohol, sulphuric acid, and sodium chromate.

In testimony whereof, we sign this specification.

JAMES D. KLINGER.  
CLETE L. BOYLE.